

June 29, 1954

S. K. TALLEY ET AL

2,682,523

LUBRICANTS

Filed May 24, 1950

3 Sheets-Sheet 1



INVENTORS:

FIG.I

S. K. TALLEY  
T. E. REAMER  
BY: *James Jodoric*  
THEIR ATTORNEY

June 29, 1954

## S. K. TALLEY ET AL LUBRICANTS

2,682,523

Filed May 24, 1950

3 Sheets-Sheet 2

EAST TEXAS SHORT RESIDUE WAX

- ① AROMATIC HYDROCARBON
  - ② NAPHTHENIC/AROMATIC HYDROCARBON
  - ③ ISOPARAFFIN /NAPHTHENIC HYDROCARBON
  - ④ STRAIGHT CHAIN PARAFFIN HYDROCARBON



FIG. II

**INVENTORS:**

S.K. TALLEY  
T.E. REAMER

BY: James Todorovic  
THEIR ATTORNEY

June 29, 1954

S. K. TALLEY ET AL

2,682,523

LUBRICANTS

Filed May 24, 1950

3 Sheets-Sheet 3

- LOW MELTING DISTILLATE PARAFFIN WAX (M.P.126°F)
- CHLORINATED LOW MELTING CHLORINATED DISTILLATE PARAFFIN WAX (M.P.126°F; 29%CI)
- HIGH MELTING POINT RESIDUE WAX (M.P.180-185°F)
- CHLORINED HIGH MELTING POINT RESIDUE WAX (M.P. 180-185°F; 29%CI)



FIG. III

INVENTORS:

S. K. TALLEY  
T. E. REAMER

BY: *James F. Talle*  
THEIR ATTORNEY

## UNITED STATES PATENT OFFICE

2,682,523

## LUBRICANTS

Samuel K. Talley, Berkeley, and Thomas E. Reamer, Albany, Calif., assignors to Shell Development Company, San Francisco, Calif., a corporation of Delaware

Application May 24, 1950, Serial No. 163,966

15 Claims. (Cl. 252—49.5)

1

2

This invention deals with the preparation and use of halogenated derivatives of high melting point hydrocarbon waxes derived from petroleum distillation residues. It especially involves the production of halogenated petroleum wax obtained from distillation residues of petroleum oils of mixed or paraffin base character which may be East Texas, Mid-Continent, Pennsylvania crudes or the like.

Generally, hydrocarbon waxes are produced (separated) from oily wax masses recovered from petroleum lubricating oil base stocks during the treatment of such lubricating oil stocks to remove therefrom materials which markedly reduce the fluidity of the oil when it is cooled to low temperatures, such as 0° C. and the like. In order to produce lubricating oils with given viscosity characteristics, the base stock is generally first separated into different fractions by distillation, under reduced pressure, and the distillate fractions, as well as the residual fraction, are subsequently "dewaxed" to remove the higher melting hydrocarbons present and to produce an oil with a suitable pour point. In the case of stocks which contain aromatic and resinous materials, these are usually extracted with a selective solvent, such as furfural, phenol, and the like, such extraction being generally carried out before the dewaxing. The dewaxing may be effected simply by chilling the waxy oil fraction to crystallize the higher melting hydrocarbons present therein, and pressing, filtering or centrifuging to separate the oil from the wax, which wax is called "slack" wax or crude wax and which is an oily wax mass of solidified hydrocarbons and liquid hydrocarbons entrained therewith. By the well-known "sweating" operation, the oils (liquid hydrocarbons) may be at least partially removed from the slack or crude wax, thereby yielding a harder wax product, the so-called "scale" wax, and a still more oily wax product, so-called "slop" wax, which is a soft wax. Essentially the same separations may be effected in the presence of an inert diluent, such as a light hydrocarbon, propane, butane, and the like, or in the presence of various organic solvents which may exert preferential solvent action for one type of hydrocarbons present over another type present, such as methylethyl ketone, acetone, benzene, toluene, and the like, and mixtures thereof, as is well known and practiced in the art, with appropriate selection of dewaxing temperatures for the waxy oil and of deoiling temperatures for de-oiling the oily wax.

The lower melting and lower molecular weight

crystalline and molecular weight paraffin waxes are obtained from the lower boiling distillate fractions, while the higher melting crystalline paraffin waxes are derived from the higher boiling distillate fractions. In the case of the residual material from the vacuum distillation used to produce the distillate lube stocks, the waxes obtained therefrom are of still higher molecular weight, but appear to be of an entirely different character, their nature being such that a mass thereof is obtained which to the unaided eye appears to have no crystalline character and to be amorphous, having somewhat plastic characteristics and having refractive indices indicating the principal components to be non-straight chain hydrocarbons and to be for the most part a mixture of isoparaffinic, naphthenic and aromatic hydrocarbons. Magnification reveals a microcrystalline structure, hence the name "microcrystalline" wax.

It is an object of this invention to produce halogenated high melting point waxes obtained from particular petroleum hydrocarbon fractions. A further object is to produce a chlorinated high molecular weight and high melting point wax material from short residue fractions of waxy petroleum base stocks. A still further object is to produce aqueous and non-aqueous emulsions containing as an essential ingredient a new halogenated, high molecular weight and high melting point hydrocarbon wax derived from short residue fractions of waxy petroleum base stocks, said emulsions having wide applicability for industrial uses. These objects will be better understood, other objects will appear and the attainment of them made clear from the description of the invention, which will be made with reference to the accompanying drawings, wherein: Figure I is a flow sheet for the process of preparing waxes of this invention; Figure II discloses the composition of waxes of this invention from which the halogenated derivatives are obtained and Figure III discloses comparative test data of waxes of this invention as against waxes well known in the art.

It has now been found that a new and novel hydrocarbon wax derivative product can be obtained by halogenating a hydrocarbon wax preferably predominating in straight-chain structure, having a melting point above 160° F. to about 225° F. and a molecular weight of from about 475 to 1000 and higher, said wax being derived from the short residue fractions of waxy base stocks, exemplified by East Texas, Mid-Continent, Pennsylvania stocks and the like.

The halogenated waxes of the invention are useful as such in metal-working operations and also in certain emulsions as will be described hereinafter.

Briefly stated, the hydrocarbon waxes and fractions thereof, from which the halogenated waxy products of this invention are made, are derived from the short residue fractions of waxy petroleum base stocks such as East Texas, Mid-Continent and Pennsylvania crudes, said waxes having a paraffinicity corresponding to a content of at least 60%, and preferably at least 80% by weight or more, thereof of straight-chain paraffin hydrocarbons, the hydrocarbon wax having a melting point of at least 160° F., and preferably above 180° F., and a molecular weight around 475 and preferably ranging from 525 to 1000.

Broadly stated, the hydrocarbon waxes, from which the novel halogenated waxes are produced, can be obtained from petroleum oils derived from different sources or localities and having different specific characteristics, the only requirement being that the oil be of a paraffinic or paraffinic-naphthenic character; that is, that it is a waxy oil and that it contain paraffinic hydrocarbons of high molecular weight, including normal and isoparaffinic hydrocarbons, with or without naphthenic hydrocarbons. Generally, the stock material is preferably a so-called mixed base oil in that it is largely paraffinic and naphthenic in character, the East Texas crudes being particularly valuable for recovering therefrom hydrocarbon waxes used to form the halogenated products of this invention.

The high molecular weight, high melting point paraffin hydrocarbon waxes useful in this invention can be recovered from a suitable base crude stock in the following manner. A crude oil such as an East Texas crude is topped to remove the lighter fractions and the topped crude oil is subjected to vacuum distillation to recover the distillate lubricating oil base stock in one or more fractions which contains the crystalline paraffin waxes well known in the art. The short residue fraction is further processed in order to recover the wax fraction thereof used to form the halogenated products of this invention by deasphalting if necessary, solvent extracting to produce a waxy, raffinate residual stock, dewaxing the deasphalted and solvent extracted short residue fraction so as to separate the wax from the oil and, if desired, fractionating said wax into various high melting point fractions, which fractions, singly or in combination, can be halogenated and utilized for a specific purpose such as for waterproofing and coating materials, electrical insulation, fire proofing, lubricating oil such as drawing oil and the like. To elucidate further, the short residue can be subjected to propane deasphalting treatment and the deasphalted short residue subjected to solvent extraction treatment with phenol or the like, and the waxy raffinate fraction further processed. This waxy raffinate is subjected to a dewaxing solvent treatment in order to recover from the waxy raffinate the so-called short residue slack or crude wax. This short residue crude wax is de-oiled as by dissolving the wax in a typical wax de-oiling solvent or solvent mixture at a rather elevated temperature and cooling the solution to a suitable temperature so as to precipitate the waxes while leaving the oily components and portions of the lower melting wax constituents dissolved in the solvent, and filtering the slurry in order to recover a primary microcrystalline wax having a melting point

of above about 160° F. This microcrystalline wax can be segregated into two wax products by dissolving it in dewaxing or de-oiling solvents at an elevated temperature and cooling the solution just sufficiently to precipitate a hard paraffin wax having a melting point above 160° F. and generally above 180° F.; a plastic microcrystalline wax with a melting point above 140° F. is recoverable from the filtrate. To form the new and novel halogenated products of this invention, the primary microcrystalline wax having a melting point above 160° F., or the plastic microcrystalline wax, or the high melting point paraffin wax recovered from the primary microcrystalline wax, as well as fractions and mixtures thereof, can be used.

In order to more clearly set forth the manner in which high melting point waxes, used to form the halogenated products of this invention, are produced, reference is made to Figure I, which is a schematic flow diagram illustrating a process of recovering waxes of this invention from suitable base stocks. For example, a topped East Texas crude oil is subject to vacuum distillation (1) to recover the distillate lubricating oil base stock contained therein, including all material which is removable at about 650° F. and 130 mm. of mercury absolute pressure. From this lubricating oil distillate can be recovered the conventional or commercial crystalline hydrocarbon wax known in the art as paraffin wax, in the manner indicated in the flow diagram by steps (7), (8), and (9). This paraffin wax is a low melting wax having a melting point range from 113° to less than 140° F. This type of low melting paraffin wax, and particularly the halogen derivatives, is clearly distinct in properties and utility to the high melting point waxes of this invention and particularly to the halogenated products thereof.

The residue fraction, if necessary, is given a propane deasphalting treatment (2) yielding a deasphalted short residue. The deasphalted short residue is then given solvent extraction treatment (4) with any suitable selective solvent, such as phenol, (3) which results in the formation of a short residue deasphalted extract and a short residue deasphalted waxy raffinate fraction. The waxy raffinate is dissolved in a dewaxing solvent or solvent mixture (4) such as the usual mixture of methylethyl ketone, benzene and toluene, the solution is chilled to about -10° F. to precipitate the waxes and filtered to recover wax from the oil. The wax is usually thoroughly washed on the filter, after which it is recovered as an oily wax, so-called short residue crude or slack wax. A representative crude wax thus produced had the following properties:

|                                      |        |
|--------------------------------------|--------|
| Sp. gr. (20/4° C.)                   | 0.8936 |
| Refractive index (90° C./D.)         | 1.452  |
| Color (ASTM D155-45T) at 100° C      | 4 1/2  |
| Dropping point (ASTM D566-42), °F    | 171    |
| Cloud point (methylethyl ketone), °F | 154    |

This short residue crude wax is de-oiled as by dissolving the wax in a typical wax de-oiling solvent or solvent mixture such as methyl isobutyl ketone or the usual dewaxing solvent mixture of methylethyl ketone, benzene and toluene (5), for example, 7 volumes of solvent to 1 volume of wax at a solution temperature of about 140° F., cooling the solution to a suitable temperature such as about 60° F. to precipitate the waxes while leaving the oily components, and a portion of the lower melting wax constituents, such as those melting up to 117° F., and recovering a primary

microcrystalline wax (a) having a melting point of about 160° F., the component parts of which are shown graphically in Figure II by areas (1), (2), (3) and (4), the molecular weights of which are above 475 and range from about 525 to 1000.

The primary microcrystalline wax (a) is segregated into two wax products by fractional crystallization (6). This is suitably accomplished by dissolving wax (a) in from about 5 to about 10, preferably 7, volumes of a suitable dewaxing or de-oiling solvent, as already described, at a suitable elevated temperature, such as about 160° F., and chilling the solution sufficient to precipitate substantially only the higher melting point waxes (b), or (c) if subsequently clay treated, and filtering the precipitated high melting point, hard paraffin wax having a melting point above about 180° F., the component parts of which are represented graphically in Figure II by the area bracketed by 180° F. The wax fraction in the solution is recovered by distilling off the solvent, or by precipitation at a still lower temperature, to produce a plastic microcrystalline wax (d), or (e) if subsequently clay treated, said wax having a melting point above 140° F. Referring to Figure II, it can be seen that the wax (b) or (c) of Figure I is the wax fraction embraced by the bracket 180° F. and consists of approximately 80% of high melting straight-chain paraffin waxes having an average melting point of about 180° F., the melting point of the lowest melting constituent thereof being about 160° F., and about 20% of a mixture of high melting isoparaffinic, naphthenic and aromatic hydrocarbons, while the remainder of the primary microcrystalline wax (a), which remainder is the plastic microcrystalline wax (d) or (e), is essentially all isoparaffinic/naphthenic (about 80%), about 3% being straight-chain paraffinic and the remainder (about 17%) being a mixture of naphthenic and aromatic hydrocarbons.

The data in Table I show the yields and properties of various high melting, essentially straight-chain paraffin waxes and of the complementary plastic waxes obtained from the de-oiled primary microcrystalline wax at various filtration temperatures.

indicating that the high melting wax was essentially pure normal paraffin wax; this wax is indicated by the bracketed 190° F. wax in Figure II. At a filtration temperature of 104° F., the high melting wax had a melting point of 182° F., and its index of refraction differed from that of the normal paraffin hydrocarbon of the same melting point by only 0.0042 unit at 90° C. The penetration of this latter high melting wax was 4 to 6 mm./10 g. at 95° F., as compared with a value of 1 to 2 mm./10 g. for the 191° F., melting point wax.

It has been found that the high-melting waxes of relatively low index of refraction, comprising essentially and substantially only high melting point, normal paraffin hydrocarbons, are recoverable from the primary microcrystalline wax, or from the entire residual slack wax, by dissolving the wax in a suitable wax (or so-called "dewaxing") solvent, such as methylethyl ketone, methyl isobutyl ketone, acetone, dichloro-diethyl ether, methyl isobutyl carbinol, and the like, or mixtures thereof, as well as mixtures of such solvents with aromatic hydrocarbons such as benzene, toluene, and the like, in a solvent to wax weight ratio of 25 from about 2:1 to about 10:1, preferably from about 5:1 to about 9:1, at a temperature at least as high as about the normal melting point of the wax being treated, and generally about 150° F. to 170° F., and cooling the solvent-wax solution to a 30 temperature from about 65° F. to about 80° F., below the desired melting point of the high melting, hard, paraffin wax which it is desired to precipitate from the solution and to recover as high melting wax. In order to recover hard wax with 35 the highest melting point, the difference between the melting point of said wax and the filtration temperature must be at a minimum, being of the order of about 65° F. or less. For each degree change desired in the melting point of the hard, high melting wax, the filtration temperature should be changed by about two degrees. In general, the filtration temperature should be about 100° F. or higher, depending on the specific properties desired for the separated wax.

45 A preferred wax from which the halogenated products of this invention can be made is the

TABLE I  
Fractionation of East Texas short residue primary  
microcrystalline wax

| Filtration Temp.,<br>° F. | Solv./Wax,<br>wt. ratio | High Melting Wax |                |                     | $n_p^{90^\circ} C.$<br>from n-P of<br>same M. P. | Plastic Wax    |                     |                   |
|---------------------------|-------------------------|------------------|----------------|---------------------|--------------------------------------------------|----------------|---------------------|-------------------|
|                           |                         | Yield            | M. P.,<br>° F. | $n_p^{90^\circ} C.$ |                                                  | M. P.,<br>° F. | $n_p^{90^\circ} C.$ | Pen. at<br>95° F. |
| 122                       | 5                       | 15               | 191            | 1.4394              | 0.0023                                           | 157            | 1.4440              | 30                |
| 111                       | 7                       | 28               | 185            | 1.4392              | 0.0036                                           | 149            | 1.4453              | 35                |
| 106                       | 9                       | 32               | 183.5          | 1.4395              | 0.0042                                           | 145            | 1.4450              | 46                |
| 104                       | 5                       | 38               | 182            | 1.4392              | 0.0042                                           | 142            | 1.4457              | 46                |
| 95                        | 5                       | 48               | 177.5          | 1.4406              | 0.0067                                           | 137            | 1.4467              | 55                |

n-P=normal paraffin.

The values given in the sixth column of Table I are for the deviation between the index of refraction as actually determined for a given wax fraction and the index of refraction of the normal (straight-chain) paraffin hydrocarbon of the same melting point as the given wax fraction, the index of refraction being determined at 90° C., utilizing the D spectral emission line of sodium. It will be seen that at a filtration temperature of 122° F., the separated high melting wax had a melting point of 191° F. and an index of refraction which differed only 0.0023 unit from the index of refraction of the normal paraffin hydrocarbon which has a melting point of 191° F., thus

65 hard, high melting hydrocarbon wax represented by (b), or (c) in Figure I, said wax having the following properties:

Melting point, ° F. 184.  
R. I. at 90° C. 1.4383.  
Density (20/4° C.) 0.9350 g./ml.  
Visc. (SUS/210° F.) 70.6.  
Needle penetration at 95°

70 F. 1.

Normal paraffin hydrocarbon, per cent. At least 80 or higher.

In order to clearly show the marked difference 75 in properties between high melting waxes such

as obtained from short residues and identified as (a) through (e) in Figure I, and paraffin waxes obtained from distillate fractions as shown in steps (7) through (9) in Figure I, an East Texas topped crude was subjected to vacuum distillation and the waxes from the short residue and waxes from distillate fractions were recovered and their properties were determined and found to be as follows:

|                                      | Wax derived from 100 SUS at 100° F. distillate (of Fig. I) | Wax derived from 250 SUS at 100° F. distillate (of Fig. I) | Residue Plastic Microcrystalline Wax (d or e of Fig. I) | Residue High Melting Paraffin Wax (b or c of Fig. I) |
|--------------------------------------|------------------------------------------------------------|------------------------------------------------------------|---------------------------------------------------------|------------------------------------------------------|
| Melting Point, ° F.                  | 125                                                        | 141                                                        | 145                                                     | 183                                                  |
| R. I. at 90° C.                      | 1.4222                                                     | 1.4300                                                     | 1.4438                                                  | 1.4403                                               |
| Needle Penetration, mm./10 at 95° F. | 34                                                         | 33                                                         | 29                                                      | 12                                                   |
| Sp. gr. at 20° C. (by displacement)  | 0.877                                                      | 0.882                                                      | 0.921                                                   | 0.934                                                |
| Oil Content (ASTM), percent wt.      | 0.5                                                        | 0.9                                                        | 1.7 (soc)                                               | 0.2                                                  |
| SUS/210° F.                          | 35.8                                                       | 41.0                                                       | 76.4                                                    | 73.5                                                 |
| Mol. Wt.                             | 347                                                        | 447                                                        | 665                                                     | 641                                                  |

In order to produce the halogenated waxes of the present invention, the short residue hydrocarbon waxes having a melting point above about 160° F., a molecular weight of at least 475 and preferably between 525 and 1000 and consisting predominantly of straight-chain hydrocarbons are halogenated by conventional means until the wax has a halogen content of at least 20% and preferably so that the wax contains a halogen content of from 25% to about 60%.

The preferred halogenating agent is gaseous chlorine and the waxes of this invention can be chlorinated by passing gaseous chlorine through the wax at just above its melting point, with or without the use of a catalyst. After chlorination it is preferable to blow the chlorinated wax with an inert gas such as nitrogen and the like. Instead of chlorinating waxes of this invention, they can be fluorinated, brominated, or the wax can be halogenated in such a manner as to contain dissimilar halogen atoms in the molecule. In all cases it is preferred that the halogen content of the halogenated high melting, high molecular weight residue hydrocarbon waxes be above 20% and preferably range from 25 to 60%, by weight.

As a specific example, a hard, high-melting (184° F.) high molecular weight (640-660), predominantly straight-chain paraffin wax was heated to about 230-248° F. and maintained at said temperature while chlorine gas was passed through the molten wax until the chlorine content was at least about 30%. The chlorinated wax was blown with nitrogen in order to remove impurities and the resulting product was a dark brown, highly viscous mass and had the following properties:

|                                |       |
|--------------------------------|-------|
| Sp. gr. (20/4° C.)             | 1.2   |
| Chlorine (percent)             | 42.2  |
| Visc. at 130° F. (centistokes) | 5061  |
| Visc. at 210° F. (centistokes) | 300.6 |
| Br. No.                        | 0.0   |
| Mol. wt.                       | 1102  |

In addition to the halogenation of the waxes of this invention by the method described above, the waxes can be halogenated (with the necessary modifications in view of the high melting wax of this invention) under conditions substantially described in U. S. Patents 2,186,916, 2,340,968, 2,372,414, 2,370,787, and 2,403,179.

Specific products of utility in accordance with this invention are:

(1) Chlorinated derivative of crude primary microcrystalline residue hydrocarbon wax having a melting point of 160-165° F. and a chlorine content of from 25 to 60%.

(2) Chlorinated derivative of a high melting predominantly straight-chain, residue, paraffin wax originally having a melting point of 180-195°

25 F. and to give a product having a chlorine content of from 25 to 60%.

(3) Fluorinated derivative of a primary microcrystalline residue hydrocarbon wax having a melting point of 160-165° F. and a fluorine content of from 20 to 60%.

(4) Fluorinated derivative of a high melting, residue, straight-chain paraffin wax having a melting point of 180-195° F. and a fluorine content of from 25 to 60%.

35 (5) 25-60% chlorinated-fluorinated derivative of a crude primary microcrystalline residue hydrocarbon wax having a melting point of 160-165° F., the chlorine content being at least 80% of the total halogen content of the wax.

(6) 25-60% chlorinated-fluorinated derivative of a high melting, residue, straight-chain paraffin wax having a melting point of 180-195° F., the chlorine content being at least 80% of the total halogen content of the wax.

45 (7) 25-60% chlorinated derivative of a mixed residue hydrocarbon wax consisting of 50%-80% of residue, straight-chain paraffin wax having a melting point of 180-195° F. and 40%-20% of a plastic microcrystalline wax having a melting point of 140-145° F.

(8) 25-60% fluorinated derivative of a mixed residue hydrocarbon wax consisting of 60%-80% of residue, predominantly straight-chain paraffin wax having a melting point of 180-195° F. and 40%-20% of a plastic microcrystalline wax having a melting point of 140-145° F.

60 The new and novel halogenated (preferably chlorinated) derivatives of high melting, high molecular weight, hydrocarbon waxes of this invention can be used, per se, or as components in various aqueous or non-aqueous media. Chlorinated hydrocarbon waxes of this invention are useful, per se, as industrial metal-working lubricants such as rolling, drawing, stamping, forging lubricants or the like, and are particularly suitable for working metals which have a negative surface charge such as stainless and other high chromium steels. They are useful as coating and rust protective agents, for fireproofing materials, in dielectric compositions, hydraulic fluids, fly-paper coating, as plasticizers, or the like. Additionally, halogenated waxes of this invention are useful as additives in cutting oil compositions, extreme pressure lubricants, grease compositions and the like.

In making improved emulsions containing halogenated hydrocarbon waxes of this invention, it is preferable to use as the emulsifying agent neutral partial esters of polyhydric alcohols and carboxylic acids, although other emulsifying agents are suitable.

The partial ester may be derived from glycerine, erythritol, pentaerythritol, mannitol, sorbitol, sorbitan, etc. The acid forming the ester with the polyhydric alcohol should have at least about 10 and preferably from about 10 to 40 carbon atoms, in the form of an aliphatic or cyclo aliphatic radical. Suitable radicals comprise, for example, those of acids such as capric, lauric, myristic, palmitic, oleic, stearic radicals, etc. Radicals such as are contained in the acids obtained from rosin or tall oil as well as naphthenic acids having the requisite number of carbon atoms are also applicable. Specific esters are: glyceryl mono- and di-oleate, glyceryl mono- and di-stearate, sorbitan mono-, and tri-oleate, sorbitan mono-, di- and tri-stearate, glyceryl mono- and di-ricinoleate, pentaerythritol mono-stearate, glycerol mono-ester of soya bean fatty acids, pentaerythritol monocaprylate, polymerized partial esters of glycol laurate, oleyl-ricinoleate, and stearate, etc. These esters may be modified by hydrogenation condensed with alkylene oxide and the like, if desired. The amount of said partial ester alcohol which is suitably used in compositions of this invention varies from about 1 to about 25% and preferably between about 5 and 20%.

In order to impart good metal wettability and thereby greatly improve the lubricating characteristic and film strength of the halogenated wax emulsion, cationic agents containing an oleophilic group should be added to the emulsion in minor amounts, such as organic amines, amides or salts of such organic nitrogen bases. Specifically preferred are long-chain aliphatic amines or amides having 8 or more carbon atoms, for instance, up to about 40 carbon atoms, in the hydrocarbon chain, such as octyl, decyl, dodecyl, tetradecyl, hexadecyl, octadecyl, octadecenyl amines or amides. Additionally, cyclic amines and alkylol amines can be used such as cyclohexyl amine, ethanolamine, diethanolamine, N-lauryl hydroxylamine, mono-oleicamide of diethylene triamine, and the like. Quaternary ammonium compounds, such as trimethyl benzyl ammonium hydroxide, cetyl piperidinium chloride, are also useful. The general formulation of wax emulsions of this invention may be represented by:

|                                                                                                                        | Broad Range  | Preferred Range |
|------------------------------------------------------------------------------------------------------------------------|--------------|-----------------|
| Chlorinated high melting residue wax (M. P. of the paraffin wax above 160° F., 20-80% Cl).                             | 3-50%-----   | 5-40%-----      |
| Emulsifiers (partial ester of a polyhydric alcohol and a monocarboxylic acid, and alkylene oxide derivatives thereof). | 1-25%-----   | 5-20%-----      |
| Cationic wetting agent: amines, amides, quaternary ammonium compounds or mixture thereof.                              | 0.7-10%----- | 0.5-5%-----     |
| Aqueous base (water)-----                                                                                              | Balance----- | Balance-----    |

The emulsions can be prepared by any suitable means such as by heating the chlorinated residue wax until suitably fluid, adding the emulsifier and cationic wetting agent and heating the mixture under constant agitation. The required amount of water is added with constant agitation and the mixture cooled to room temperature. Instead of adding the emulsifier to the

molten chlorinated wax, it can be admixed with the water and introduced into the fluid chlorinated wax in that manner. The product is dispersible in water and other aqueous media and excellent lubricants are obtained when the base emulsion is used with water in the ratio of 1:2 to 1:10.

Excellent drawing lubricants utilizing halogenated waxes of this invention are illustrated by the following examples:

|    | EXAMPLE I                                                                                                 | Per cent |
|----|-----------------------------------------------------------------------------------------------------------|----------|
| 15 | Chlorinated high melting point hydrocarbon wax (180-185° F. M. P. of the paraffin wax and 25-35% Cl)----- | 40       |
|    | Sorbitan monooleate-----                                                                                  | 4        |
|    | Polyoxyethylene sorbitan monooleate-----                                                                  | 4        |
|    | Lauryl amine-----                                                                                         | 2        |
| 20 | Water-----                                                                                                | Balance  |

|    | EXAMPLE II                                                                                                  | Per cent |
|----|-------------------------------------------------------------------------------------------------------------|----------|
| 25 | Chlorinated primary microcrystalline wax (160-165° F. M. P. of the microcrystalline wax and 30-40% Cl)----- | 40       |
|    | Sorbitan monooleate-----                                                                                    | 4        |
|    | Polyoxyethylene sorbitan monooleate-----                                                                    | 8        |
|    | Stearyl amine-----                                                                                          | 2        |
| 30 | Water-----                                                                                                  | Balance  |

|    | EXAMPLE III                                                                                                  | Per cent |
|----|--------------------------------------------------------------------------------------------------------------|----------|
| 35 | Chlorinated high melting point hydrocarbon wax (180-185° F. M. P. of the hydrocarbon wax and 25-35% Cl)----- | 35       |
|    | Mineral oil-----                                                                                             | 5        |
|    | Glycerol monooleate-----                                                                                     | 4        |
|    | Polyoxyethylene sorbitan monooleate-----                                                                     | 4        |
|    | Dodecyl amine-----                                                                                           | 2        |
| 40 | Water-----                                                                                                   | Balance  |

|    | EXAMPLE IV                                                                                                      | Per cent |
|----|-----------------------------------------------------------------------------------------------------------------|----------|
| 45 | Chlorinated high melting point residue hydrocarbon wax (M. P. of the hydrocarbon wax, 180-185° F., 40% Cl)----- | 30       |
|    | Sorbitan monooleate-----                                                                                        | 2        |
|    | Polyoxyethylene sorbitan monooleate-----                                                                        | 4        |
|    | Abietyl amine-----                                                                                              | 3        |
| 50 | Water-----                                                                                                      | Balance  |

|    | EXAMPLE V                                                                                                   | Per cent |
|----|-------------------------------------------------------------------------------------------------------------|----------|
| 55 | Chlorinated high melting point residue hydrocarbon wax (M. P. of hydrocarbon wax, 180-185° F., 40% Cl)----- | 35       |
|    | Mannitan monolaurate-----                                                                                   | 2        |
|    | Polyoxyethylene mannitan monolaurate-----                                                                   | 4        |
|    | Oleyl amine-----                                                                                            | 3        |
| 60 | Water-----                                                                                                  | Balance  |

|    | EXAMPLE VI                                                                              | Per cent |
|----|-----------------------------------------------------------------------------------------|----------|
| 60 | Chlorinated high melting point residue hydrocarbon wax (M. P. 160-165° F., 30% Cl)----- | 40       |
|    | Pentaerythritol monocaprylate-----                                                      | 4        |
|    | Polyoxyethylene sorbitan monostearate-----                                              | 4        |
|    | Stearic acid amide-----                                                                 | 4        |
| 65 | Water-----                                                                              | Balance  |

In order to show the marked superiority of halogenated waxes of this invention, neat or in emulsion form, as lubricants for drawing of metals the following materials were tested by the friction draw test machine in the following manner. Stainless steel metal strips were lubricated with materials being tested and the lubricated metal strip was pulled between two opposing flat dies under a constant load. The tensile force required to draw the metal sheet between the

## 11

dies was measured in conjunction with the known normal force on the dies and from these values the coefficient of friction was determined.

## COMPOSITION TESTED

- (1) Chlorinated high melting residue hydrocarbon wax (M. P. of the wax 180-185° F., 25-30% Cl)
- (2) Chlorinated low melting distillate paraffin wax (M. P. of the wax 126° F., 29% Cl)
- (3) Emulsion as defined by Example I
- (4) Emulsion as defined by Example I, except that a chlorinated distillate paraffin wax (M. P. of the wax 126° F. and 29% Cl) was substituted for the chlorinated residue wax
- (5) High melting residue hydrocarbon wax (M. P. 180-185° F.)
- (6) Low melting distillate paraffin wax (M. P. 126° F.)

Some of the test results are represented graphically in Figure III and the superiority for compositions of this invention over those containing the conventional halogenated paraffin waxes can be clearly noted. In Figure III, low coefficient of friction at high normal loads indicates a superior lubricant.

In actual plant operation, stainless steel tubes having an initial diameter of 1 1/4", oxidized surface finish, were drawn with the aid of chlorinated waxes of this invention per se or neat, and in emulsion form, and the results compared with commercial lubricants, the results being tabulated below:

| Composition                                                                                                                                                                      | 36% Reduction                                              | Speed (ft./min.) |
|----------------------------------------------------------------------------------------------------------------------------------------------------------------------------------|------------------------------------------------------------|------------------|
| (1) Chlorinated high melting point residue hydrocarbon wax (M. P. of the wax 180-185° F., 30-40% Cl).                                                                            | Smooth draw, no rod chatter, normal deposit in mandrel.    | 18.75 to 37.5.   |
| (2) Chlorinated distillate paraffin wax (M. P. of the wax, 124° F., 40% Cl).                                                                                                     | Severe stick-slip, could not be drawn.                     | 18.75.           |
| (3) Composition Example IV of present invention.                                                                                                                                 | Smooth draw, no chatter in die, normal deposit in mandrel. | 18.75.           |
| (4) Composition: Chlorinated distillate wax (M. P. of wax 124; Cl 42%); Remainder same as Ex. IV—Sorbitan monooleate, Polyoxyethylene sorbitan, monooleate, Stearylamine, Water. | Smooth draw for 8 ft. then severe chatter noted.           | 18.75.           |

The vehicles to which halogenated waxes of this invention can be added, generally in minor amounts of from 3 to 49% and preferably from 5 to 25% are suitably any substantially neutral vehicle of polar and non-polar character such as water, water emulsions, natural, synthetic and/or mineral oils, e. g. castor oil, lard oil, mineral oil, greases, polymeric olefins and copolymers such as alkylene glycolalkylene oxide copolymer, natural and synthetic resins, etc.

To compositions containing the halogenated derivative of a high melting point wax of this invention can be added, e. g., non-metallic detergents such as the phosphatides, lecithin and cephalin, certain fatty oils as rapeseed oils, voltolized fatty or mineral oils or lanolin, sulfonates, metal stearate e. g. Ca or Al stearate, phenates (halo-waxes), and the like.

Anti-oxidants can be added to halogen-waxes of this invention such as, for example, alkyl phenols such as 2,4,6-trimethyl phenol, 2,4-di-methyl-6-tertiary-butyl phenol, 2,6-di-tertiary-butyl-4-methyl-phenol, and the like; amino phenols as benzyl amino phenols; amines such as dibutyl-phenylene diamine, diphenyl amine, 70

phenyl beta - naphthylamine, phenyl - alpha - naphthylamine and dibutylamine.

Corrosion inhibitors or anti-rusting compounds may also be combined with the halogen waxes, such as dicarboxylic acids of 16 and more carbon atoms, e. g., octadecenyl- and octadecylsuccinic acid, alkali metal and alkaline earth metal salts of sulfonic acids (petroleum sulfonic acids) and fatty acids, organic compounds containing an acidic radical in close proximity to a mercapto, nitrile, nitro or nitroso group (e. g., alpha cyano stearic acid).

Additional ingredients may comprise oil-soluble urea or thiourea derivatives, e. g., urethanes, allophanates, carbazides, carbazones, etc., polyisobutylene polymers, unsaturated polymerized esters of fatty acids and monohydric alcohols and other high molecular weight oil-soluble compounds.

Depending upon the additional additive used and conditions under which it is used, the amount of additive used may vary from 0.1% to 2% or higher. However, substantial improvement is obtained by using amounts ranging from 15 0.1% to 0.5% in combination with the halogenated high melting point waxes of this invention.

Compositions of this invention can be applied to and removed from the surfaces to which they have been applied by any suitable means such as are well known in commercial practice.

We claim as our invention:

1. An aqueous emulsion metal-working lubricating concentrate composition containing from 3 to 50% of a halogenated high melting residue hydrocarbon wax containing 20-60% halogen, the hydrocarbon wax having a melting point of

55 at least 160° F., a molecular weight above 475, and consisting of at least 60% normal straight-chain hydrocarbons and the remaining constituents being high melting isoparaffinic and naphthenic hydrocarbons; from about 1% to about 25% of an ester selected from the group consisting of an ester of a polyhydric alcohol and a carboxylic acid and a polyalkylene glycol ether of a partial ester of a polyhydric alcohol and a carboxylic acid; from about 0.7% to 10% of an organic nitrogen-containing compound having a hydrocarbon chain of from 8 to 18 carbon atoms selected from the group consisting of an aliphatic amine, and an aliphatic amide; and the balance being water.

60 2. An aqueous emulsion metal-working lubricating concentrate composition containing from 3 to 50% of a halogenated high melting residue hydrocarbon wax containing 20-60% halogen, the hydrocarbon wax having a melting point of at least 180° F., a molecular weight above 600, and consisting of at least 80% normal straight-chain hydrocarbons and the remaining constituents being isoparaffinic and naphthenic hydrocarbons; from about 1% to about 25% of an ester of a

polyhydric alcohol and an aliphatic monocarboxylic acid; from about 0.7% to 1% of a long-chain aliphatic amine having a hydrocarbon chain of from 8 to 18 carbon atoms; and the balance being water.

3. An aqueous emulsion metal-working lubricating concentrate composition containing from 3 to 50% of a chlorinated high melting residue hydrocarbon wax containing 20-60% chlorine, the hydrocarbon wax having a melting point of at least 180° F., a molecular weight above 600, and consisting of at least 80% normal straight-chain hydrocarbons and the remaining constituents being isoparaffinic and naphthenic hydrocarbons; from about 1% to about 25% of an ester of a polyhydric alcohol and an aliphatic monocarboxylic acid; from about 0.7% to 1% of a long-chain aliphatic amine having a hydrocarbon chain of from 8 to 18 carbon atoms; and the balance being water.

4. An aqueous emulsion metal-working lubricating concentrate composition containing from 3 to 50% of a fluorinated high melting residue hydrocarbon wax containing 20-60% fluorine, the hydrocarbon wax having a melting point of at least 180° F., a molecular weight above 600, and consisting of at least 80% normal straight-chain hydrocarbons and the remaining constituents being isoparaffinic and naphthenic hydrocarbons; from about 1% to about 25% of an ester of a polyhydric alcohol and an aliphatic monocarboxylic acid; from about 0.7% to 1% of a long-chain aliphatic amine having a hydrocarbon chain of from 8 to 18 carbon atoms; and the balance being water.

5. An aqueous emulsion metal-working lubricating concentrate composition containing from about 5 to 40% of a chlorinated high melting residue hydrocarbon wax containing approximately 20-40% chlorine, the hydrocarbon wax having a melting point above 180° F., a molecular weight above 600, and consisting essentially of a mixture of normal straight-chain hydrocarbons and isoparaffinic hydrocarbons, the normal straight-chain hydrocarbons constituting about 80% of the wax mixture; from 5 to 20% of sorbitan monooleate, from 0.5 to 5% of a long-chain aliphatic amine having a hydrocarbon chain of from 8 to 18 carbon atoms; and the balance being water.

6. An aqueous emulsion metal-working lubricating concentrate composition containing from about 5 to 40% of a chlorinated high melting residue hydrocarbon wax containing approximately 20-40% chlorine, the hydrocarbon wax having a melting point above 180° F., a molecular weight above 600, and consisting essentially of a mixture of normal straight-chain hydrocarbons and isoparaffinic hydrocarbons, the normal straight-chain hydrocarbons constituting about 80% of the wax mixture; from 5 to 20% of sorbitan monooleate, from 0.5 to 5% of laurylamine; and the balance being water.

7. An aqueous emulsion metal-working lubricating concentrate composition containing from about 5 to 40% of a chlorinated high melting residue hydrocarbon wax containing approximately 20-40% chlorine, the hydrocarbon wax having a melting point above 180° F., a molecular weight above 600, and consisting essentially of a mixture of normal straight-chain hydrocarbons and isoparaffinic hydrocarbons, the normal straight-chain hydrocarbons constituting about 80% of the wax mixture and the balance of said wax mixture consisting predominantly of a mix-

ture of naphthenic and aromatic hydrocarbons; from 5 to 20% of polyoxyethylene sorbitan monooleate, from 0.5 to 5% of laurylamine; and the balance being water.

5 8. An aqueous emulsion metal-working lubricating concentrate composition containing from about 5 to 40% of a chlorinated high melting residue hydrocarbon wax containing approximately 20-40% chlorine, the hydrocarbon wax having a melting point above 180° F., a molecular weight above 600, and consisting essentially of a mixture of normal straight-chain hydrocarbons and isoparaffinic hydrocarbons, the normal straight-chain hydrocarbon constituting about 15 80% of the wax mixture and the balance of said wax mixture consisting predominantly of a mixture of naphthenic and aromatic hydrocarbons; from 5 to 20% of polyoxyethylene sorbitan monooleate, from 0.5 to 5% of abietylamine; and the balance being water.

20 9. An aqueous emulsion metal-working lubricating concentrate composition containing from about 5 to 40% of a chlorinated high melting residue hydrocarbon wax containing approximately 25 20-40% chlorine, the hydrocarbon wax having a melting point above 180° F., a molecular weight above 600, and consisting essentially of a mixture of normal straight-chain hydrocarbons and isoparaffinic hydrocarbons, the normal straight-30 chain hydrocarbon constituting about 80% of the wax mixture and the balance of said wax mixture consisting predominantly of a mixture of naphthenic and aromatic hydrocarbons; from 5 to 20% of polyoxyethylene sorbitan monooleate, from 0.5 to 5% of stearylamine; and the balance being water.

35 10. An aqueous emulsion metal-working lubricating concentrate containing the following constituents in approximately the following proportions:

|                                                  | Per cent |
|--------------------------------------------------|----------|
| Hydrocarbon wax residue as defined in<br>claim 5 | 30       |
| Sorbitan monooleate                              | 2        |
| Polyoxyethylene sorbitan monooleate              | 4        |
| Stearyl amine                                    | 3        |
| Water                                            | Balance  |

50 11. An aqueous emulsion metal-working lubricating concentrate containing the following constituents in approximately the following proportions:

|                                                  | Per cent |
|--------------------------------------------------|----------|
| Hydrocarbon wax residue as defined in<br>claim 5 | 30       |
| Sorbitan monooleate                              | 2        |
| Polyoxyethylene sorbitan monooleate              | 4        |
| Abietylamine                                     | 3        |
| Water                                            | Balance  |

60 12. An emulsion consisting essentially of the composition of claim 1 and additional water in the ratio of from 1:2 to 1:10, respectively.

65 13. An emulsion consisting essentially of the composition of claim 2 and additional water in the ratio of from 1:2 to 1:10, respectively.

70 14. An emulsion consisting essentially of the composition of claim 10 and additional water in the ratio of from 1:2 to 1:10, respectively.

15. An emulsion consisting essentially of the composition of claim 11 and additional water in the ratio of from 1:2 to 1:10, respectively.

15

References Cited in the file of this patent  
 UNITED STATES PATENTS

| Number    | Name           | Date           |
|-----------|----------------|----------------|
| 1,948,194 | Williams       | Feb. 20, 1934  |
| 2,119,149 | Bishop         | May 31, 1938   |
| 2,130,952 | Hardie et al.  | Sept. 20, 1938 |
| 2,420,328 | Shipp et al.   | May 13, 1947   |
| 2,420,329 | Shipp et al.   | May 13, 1947   |
| 2,496,115 | Burford et al. | Jan. 31, 1950  |
| 2,521,626 | Benning        | Sept. 5, 1950  |
| 2,524,017 | Hance et al.   | Sept. 26, 1950 |

16

Number  
 2,560,148

Name  
 Arabian

Date  
 July 10, 1951

## FOREIGN PATENTS

| Number  | Country       | Date         |
|---------|---------------|--------------|
| 569,348 | Great Britain | May 18, 1945 |

## OTHER REFERENCES

"Atlas Spans and Tweens," Atlas Powder Co.,  
 Wilmington, Del. Reprinted June 1945. Copy  
 in Div. 64.